

March 15, 1927.

1,620,813

J. D. FORRESTER

PROCESS OF MAKING ASPHALTIC ROAD MATERIAL

Filed Nov. 30, 1925



INVENTOR.  
John D. Forrester,  
BY  
Thomas E. Scafield,  
ATTORNEY.

## UNITED STATES PATENT OFFICE.

JOHN D. FORRESTER, OF KANSAS CITY, MISSOURI, ASSIGNOR TO PETER J. McINERNEY,  
OF DALLAS, TEXAS.

## PROCESS OF MAKING ASPHALTIC ROAD MATERIAL.

Application filed November 30, 1925. Serial No. 72,205.

This invention relates to improvements in a process for producing asphaltic road material, and refers more particularly to a process by means of which a material is produced which may be easily worked and is of a slushy consistency when laid and is further adapted to be laid cold, producing a compact non-rolling pavement.

Among further objects of the invention are, to provide a process for making an asphaltic mix adaptable for use both in the base and binder course and by varying the size of the aggregate it may be as well used in top course and surfacing for patchwork or generally in the road making art. The invention consists primarily in the combination or incorporation of an asphaltic binder intimately bonded with a crushed stone aggregate, the stone having been first dried to produce a better adhesion between the binder material and the mineral matter and a solvent or relatively light hydrocarbon being mixed with the asphaltic binder prior to its combination with the mineral aggregate to increase the fluidity of the binder and produce a mix which may be worked cold and shipped for considerable distances without setting or becoming congealed to the extent that it is difficult to remove the same from open-topped cars.

This invention is a continuation in part of a prior application Serial No. 39,815, filed June 26, 1925.

The process of combining an asphaltic binder with a mineral aggregate to form an asphaltic concrete is well known in the art. Furthermore, it is a well known practice to heat the mineral aggregate to drive off moisture contained therein, this moisture having the effect of preventing the proper contact and adhesion between the mineral aggregate and the asphalt. Furthermore, it is common practice to use a solvent or a relatively light fluid hydrocarbon which is combined with the stone and which is described as having the particular advantageous properties, not only in reducing the fluidity of the hydrocarbon binder, but also in its ability to produce a better adhesion between the mineral aggregate and binder. Furthermore, in some instances it has been contended that there is a certain amount of saponification produced. This particular phase of the prior art is, however, somewhat doubtful.

In recognizing the prior art, particular attention has been given to the Amies patents:

The novelty and improvement in the present invention as distinguished from this prior art lies, however, in the fact that it has been found that by first combining the solvent or light hydrocarbon with the asphalt instead of mixing the solvent with the stone, much better results in the final product and a much better mix from every standpoint is produced. Furthermore, it has been found an advantage to remove from the crushed stone aggregate what is termed as the "fines" or the smaller granular particles comprising primarily an impalpable dust which, if permitted to remain and form a part of the mix, facilitates the movement of the pavement when laid, producing rolling and preventing to a great extent the rigid interlocking of the angular surfaces of the crushed stone.

The single figure is a side diagrammatic view of an apparatus for heating the aggregate to remove the moisture with a blower connection for eliminating the fines from the aggregate.

One (1) is a retort rotatable upon the trunnions. The trunnions are in turn supported by suitable standards 3. Four (4) is a hopper, the discharge end of which is connected to a chute 5,—the latter inserted in the end of the retort by means of which the aggregate is introduced; 6 is a burner fuel, which may be either gas or oil, inserted in the end of the retort and receiving its air supply either directly from the atmosphere or through the duct 7 which has communication with the dust separator or arrester 8; 9 is a blower fan adapted to force a current of air through the perforations 10 in the retort in order to drive the fines or dust particles through the pipe 11 to the dust arrester 85 where the dust is collected by gravitational deposition in the bottom thereof while the clean air passes in a course shown by the arrows into the top of the duct 7 and thence back into the retort, or it may be exhausted 90 through an auxiliary line 12 controlled by a damper 13. Over the open discharge end of the retort is held in place a stationary baffle 14 covering the greater part of the discharge end of the retort and preventing 95 short-circuiting of the air discharged from the blower fan 9 through the holes of the retort. This baffle element causes the dust

laden air to pass into the duct 11 and thence into the dust arrester in place of being discharged through the end of the retort. The lower portion of the element 14 is cut away 5 to permit the aggregate to pass into a storage bin or the boot of an elevator not shown. In operation, the mineral aggregate is introduced to the hopper 4 from any convenient source and is thence charged to the 10 rotating retort 1 where it is subjected to the rolling and tumbling action of the retort in its rotation accompanied by additional mixing action produced by obstructions or ribs 15 positioned above the interior of the 15 retort. This rotating retort is preferably inclined towards its discharge end so that the stone aggregate works along while during this rotation of the aggregate and mixture, there is introduced to the retort heat supplied by means of the burner 6. The temperature on the interior of the retort is controlled to eliminate any moisture contained in the stone. Normally, temperatures of 20 500° F. or more are sufficient. The retort 25 is supported, as described, by means of the trunnion bearings 2 while rotative motion is imparted by means of a driving gear 16 meshing with a girth gear 17 attached to the periphery of the retort. The driving 30 gear is mounted upon a shaft 18 which is driven from any suitable source of power by means of the pulley 19.

The stone aggregate introduced to the hopper 4 is first properly graded to contain 35 the proper percentage of mineral matter of the size best adapted to the purposes to which the aggregate is to be used. On discharge from the retort, and after elimination of the fines, this mineral aggregate— 40 which may consist of crusher-run stone, either limestone, granite, crushed gravel or other adaptable mineral matter—is in condition to be combined with the binder in a suitable mixer such as a pug mill. Normally, for the binder course, stone ranging 45 from one and one-fourth inches to one-fourth inch, properly graded, is satisfactory. For the top course or surfacing, the mineral aggregate must be graded accordingly with 50 a greater percentage of the smaller stone.

The asphalt specifications will vary with 55 climatic conditions. Through the South, asphalt penetration will range from 60 to 70, while in the North, penetration is considerably greater,—in the vicinity of 95. The ductility, in any cases, should not be materially under 85 at 77° F. The asphaltic material may be either natural asphalt or a petroleum residue,—the latter being more 60 commonly utilized at the present time due to its cheapness and better adaptability to this type of mixture.

The asphalt is prepared by heating in a 65 body to a liquid condition. The solvent is then introduced to the asphaltic body by

supplying the latter to the bottom of the asphaltic body while subjecting the asphaltic binder to continuous agitation. The solvent may be added through a hollow stirring device through which the solvent flows and 70 is introduced by being discharged into the bottom of the asphaltic body from the end of the stirring device or separate mechanical agitators may be used to keep the asphaltic body in agitation while the solvent or light 75 hydrocarbon is introduced through a perforated pipe seated in the bottom of the mixer, the perforations being so arranged that the solvent is evenly distributed throughout. The asphalt is normally heated 80 to temperature ranges of 250° to 325° F.,—the temperatures depending primarily upon the character of the asphalt and the nature of the solvent, it being understood that the asphalt should not be heated above the flash 85 point of the particular solvent used. If a relatively volatile solvent is used, the temperatures should be considerably lower than when a solvent of a less volatile character is to be combined with the asphalt. The 90 nature of the solvent will depend primarily upon the distance the mix is to be transported before laying. Such light hydrocarbons as naphtha, kerosene, benzine, or similar unrefined relatively volatile products, are used.

After the solvent has been thoroughly incorporated into the asphalt, increasing materially its fluidity to a degree that it may be readily combined and intimately mixed 100 with the aggregate, there is also added a filler material such as pulverized slate, shale, lime stone dust or hydraulic cement. This filler has the quality of maintaining the asphalt in a relatively solid condition after it 105 has been laid or set upon the road. Even should the pavement be subjected to relatively high temperatures, which normally would produce flowing of the asphaltic binder, the filler material keeps the asphalt in 110 a bonded condition by supplying tiny granular particles which serve to bond the asphalt into a unitary mass. The mixture of asphaltic binder, solvent and filler material, which we may consider as our binder-mix, is 115 then added to the stone aggregate from which have been removed the fines, as explained. This combination is then thoroughly agitated or mixed together in a pug mill to produce thorough contact of the binder 120 with all of the aggregate material. Heretofore, where it was the practice to add the solvent to the crushed stone or subsequently admix the binder substance, oftentimes there were considerable portions of the aggregate which received no adequate covering of the binder substance and, as a consequence, the complete bond acquired by the present process was not possible. Furthermore, the 125 filler material was heretofore added during 130

the combination of the binder and aggregate tending to limit the distribution of the filler to concentrated areas of the aggregate. The practice of adding the filler and intimately combining it with the binder mix before mixing the binder with the aggregate eliminates the difficulty of isolating the filler material to concentrated regions in the aggregate.

10 As mentioned heretofore, the elimination of the fines or dust from the aggregate eliminates an impalpable powder which heretofore has had the effect of preventing complete adhesion between the asphalt and stone aggregate,—in fact, the powder acts as a glaze which the asphaltic binder was unable to penetrate. Furthermore, the fines present in the stone aggregate facilitated the rocking of the stone upon the binder and rolling

15 of the pavement, preventing rigid interlocking of the angular surfaces of the crushed stone. As described, the combination may be used either for binder course, top course, or for road surfacing,—the difference being

20 primarily in the size of the stone aggregate employed.

I claim as my invention:

1. A process of making asphaltic road material, comprising the steps of properly grading a mineral aggregate, heating the same to dryness, separately heating an asphaltic binder and adding a hydrocarbon solvent to increase its fluidity, incorporating into the asphalt mix while hot a filler comprising an argillaceous material and intimately combining the final asphaltic mixture with the dried mineral aggregate.
2. A process, such as that described in claim 1, in which the filler material consists of hydraulic cement.
3. A process, such as that described in claim 1, in which the filler material constitutes not less than one-half percent or more than one percent of the total weight of the mix.
4. A process, such as that described in claim 1, in which the solvent is added to the asphaltic binder by introducing the former under pressure into the bottom of the asphaltic body.

JOHN D. FORRESTER.